

# United States Patent [19]

Dollinger

[11] 3,904,727

[45] Sept. 9, 1975

[54] **METHOD OF PELLETING CARBON BLACK**

[75] Inventor: **Robert E. Dollinger, Hurst, Tex.**

[73] Assignee: **Phillips Petroleum Company, Bartlesville, Okla.**

[22] Filed: **Oct. 9, 1973**

[21] Appl. No.: **404,636**

## Related U.S. Application Data

[63] Continuation-in-part of Ser. No. 248,312, April 27, 1972, Pat. No. 3,779,683.

[52] U.S. Cl. .... **264/117; 23/314; 425/222**

[51] Int. Cl. .... **C09c 1/58**

[58] Field of Search .... **264/117, 327, 169; 23/313, 23/314; 259/DIG. 18, DIG. 22; 432/107; 425/222**

## [56] References Cited

### UNITED STATES PATENTS

3,186,928 6/1965 Keaton et al. .... **264/117**  
3,333,038 7/1967 Walenciak .... **264/117**

|           |        |             |         |
|-----------|--------|-------------|---------|
| 3,459,844 | 8/1969 | Cole.....   | 264/117 |
| 3,493,350 | 2/1970 | Howard..... | 23/314  |
| 3,528,785 | 9/1970 | Dingus..... | 264/117 |

Primary Examiner—Robert F. White

Assistant Examiner—T. E. Balhoff

[57]

## ABSTRACT

A method of pelletizing particulate solids employing a pelleteer having separate upper and lower jackets by means of which the upper and lower sections of the pelleteer can be maintained at different operating temperatures. In one embodiment of the invention, the wall of the pelleteer which comprises the inner wall of the jackets is adapted with apertures through which that material introduced into the jacket to heat the wall of the pelleteer is brought into contact with the material adhering to the inner wall of the pelleteer to remove the adhering material therefrom.

5 Claims, 3 Drawing Figures



PATENTED SEP 9 1975

3,904,727



**METHOD OF PELLETING CARBON BLACK**

This is a continuation-in-part of application Ser. No. 248,312 filed Apr. 27, 1972, now U.S. Pat. No. 3,779,683.

This invention relates to the pelleting of particulate solids.

In one of its more specific aspects this invention relates to the pelleting of carbon black.

The pelleting of particulate solids in pin-type pelleters is well known. For example, the pelleting of carbon black is disclosed in U.S. Pat. No. 3,607,086. Generally, pelleting is done in a horizontally-positioned chamber adapted with mixing means, usually a horizontally disposed pinned shaft, and conduit means for introducing the particulate solid to be pelleted and a pelleting agent. During the pelleting process, the solid is contacted by the pins as the shaft rotates and the particles are conveyed from their point of entrance to the exit of the chamber during which time the particles are agglomerated into pellets.

Among those materials employed in pelleting can be various pelleting agents, usually liquids, which facilitate the pelleting of the solids. Inasmuch as the pins on the rotating shaft almost contact the inner surface of the pelleteer, the action of the pins tends to establish a thin layer of solids on the inner wall of the pelleteer. This layer retards the rotation of the shaft, causes pin wear, and increases power requirements to rotate the shaft. The method of this invention is directed towards the solution of this problem.

According to this invention, a method of pelleting particulate solids is provided in which a particulate solid is agitated within a walled chamber, the pelleteer, in the presence of a liquid to pellet the solid and to cause a portion of the solid to adhere with the pelleting liquid to the inner wall of the chamber. At least one liquid or gaseous fluid is introduced into at least one jacket contacting the outer wall of a portion of the chamber, to vaporize at least a portion of the liquid contained in the solids adhering to the corresponding inner wall of the chamber and to heat the adhering solids. This heating is believed to remove some of the liquid from the adhering solids and to cause the solids to shrink. This shrinkage, in turn, causes the adhered solids to be removed from the corresponding inner wall of the chamber. The solids are recovered as pellets from the pelleteer.

By removing the adhering layer of particulate solids from the wall of the pelleteer, pin wear is reduced and power requirements to rotate the shaft are decreased.

In one embodiment of this invention, the lower section of the pelleteer of the upper section of the pelleteer is heated.

In another embodiment of this invention, both the upper and lower sections are heated to like, or different temperatures, as desired. Either the upper section or the lower section can be heated to the higher temperature.

In another embodiment of this invention, that fluid introduced into the jackets adjacent either the upper or lower section of the pelleteer is passed through apertures in the wall or walls of the pelleting chamber and into contact with the layer of solids adhering to the inner wall of the pelleteer, under constant or pulsating pressure, to remove at least a portion of the solids from the wall.

In the preferred embodiment of the invention, the lower section of the pelleteer is heated to an elevated temperature by the introduction of a high-temperature fluid into that jacket associated with the lower section of the pelleteer. The fluid is introduced from the lower jacket through the apertured lower wall into contact with the solids adhering to the lower inner wall of the pelleteer. A fluid at a lower temperature is introduced into that jacket in association with the upper section of the pelleteer. This fluid is not, however, passed through apertures into the upper section of the pelleteer.

The method of this invention is applicable to all pelletable solids and pelleting agents, pelleteers, and pelleting procedures. It is particularly suited for the pelleting of carbon black and will be discussed hereinafter as applied thereto without intending to limit the invention to that process.

Any suitable fluid can be introduced into the jackets and, optionally, through the apertures of the pelleteer wall. Such fluids include steam, air, nitrogen and flue gas which can be employed at any desired temperature, elevated temperatures being attained by preheating. Preferably, a hot liquid is employed when only heating of the pelleteer wall is required and a gaseous fluid is employed when the fluid is passed through apertures in the wall into contact with the adhering solids.

This invention will be more easily understood by referring to the attached drawing in which;

FIG. 1 is a view in elevation of apparatus suitable for employment in the invention and in which;

FIG. 2 is a cross-sectional view of the apparatus in which the wall of the pelleteer is not apertured;

FIG. 3 is a cross-sectional view of one embodiment in which both walls of the pelleteer are apertured.

Referring now to FIGS. 1 and 2 there is shown pelleteer 1 adapted with chamber 2 into which flocculent carbon black is introduced through inlet conduit 3 and from which wet carbon black pellets are removed through exit conduit 4. Chamber 2 is adapted with shaft 5 on which a multiplicity of pins 6 are positioned, only a portion of the pins being shown for simplicity. The shaft is rotated by conventional drive means 7. For the introduction of pelleting agents, any number of conduits means 9, which can enter the chamber at any desired location, are provided. The chamber comprises an upper section 10 and a lower section 11 which can be adapted for flanging by means of flanges 12 as shown in FIGS. 2 and 3.

Positioned around the outer periphery of sections 10 and 11 are separate upper and lower heat exchange zones, or jackets, 13 and 13' into which a fluid or fluids are introduced through conduit means 14 and 14', the fluids being removed from the jacket through conduits 15 and 15', respectively. Upon introduction of a hot fluid into the jackets, the inner surfaces 20 and 20' of sections 10 and 11 are heated with the result that the wet black cake which is adhered thereto becomes heated. As a result, vapor is produced from at least a portion of the liquid which is present in the cake, and the cake tends to shrink and be dislodged from the wall.

FIG. 3 is another embodiment of the invention having apertures 16 and 16' in the wall of the chamber. Apertures 16 can be positioned in wall 20 surrounding the upper zone 10 of the chamber and apertures 16' can be positioned in wall 20' surrounding lower zone 11, although only a single set of apertures can be employed. In this embodiment the fluid charged to the an-

nular heat exchange zones 13 and 13' can enter the chamber 2 via apertures 16 and 16' to dislodge the cake from the inner periphery of the wall.

The following examples illustrate the method of the invention.

In both examples, the pelleter chamber is 24 inches in diameter and 9 feet in length and a conventional aqueous solution containing 1 weight percent molasses is employed.

In Example I, apertures are provided in the lower wall of the pelleter. These apertures are about 1/32 inches in diameter, the total area of the apertures being about 0.01 sq. foot. Example I illustrates the preferred embodiment of the invention.

In Example II, no apertures are provided in either the upper or the lower section of the pelleter wall. Pre-heated air is introduced into both the upper and lower jackets at different temperatures to maintain a temperature differential of about 30°F between the upper and lower sections of the pelleter.

|                                |      |
|--------------------------------|------|
| Pelleter Shaft Speed, RPM      | 250  |
| Wet Pellet Production, No./hr. | 6000 |
| Pellet Temperature, °F         | 195  |
| Cake Removal, No./hr., est.    | 40   |

From the above it will be seen that if the bottom zone of the pelleter is maintained above the boiling point of the pelleting liquid and the top zone is maintained less than the boiling point of the pelleting liquid, the adhering cake can be removed. Usually the lower portion of the pelleter will be maintained about 5° to 30°F above the boiling point of the pelleting liquid and the upper portion of the pelleter will be maintained about 5° to 10° below the boiling point of the pelleting liquid although any desired differential temperature can be employed.

It will be evident from the foregoing that various modifications can be made to the method of this invention. Such are considered, however, to be within the scope of the invention.

What is claimed is:

1. A method for forming pellets from a particulate solid comprising the steps of:

- A. agitating said particulate solid within a walled chamber having an upper portion and a lower portion in the presence of a pelleting liquid whereby there are formed pellets of said solid and a layer consisting of a mixture of pelleting liquid and solids adhering to the inner walls of the lower portion of said chamber;
- B. contacting the lower portion of said walled chamber with a gaseous fluid having a temperature sufficient to heat said lower portion to a temperature above the temperature of the upper portion;
- C. passing a portion of said gaseous fluid through the inner wall of at least said lower portion of said walled chamber and into the interior thereof so as to bring said gaseous fluid into contact with at least a portion of said pelleting liquid in said layer of pelleting liquid and solids so as to vaporize at least a portion of said liquid so as to thereby cause said layer to be removed from the lower portion of said walled chamber; and thereafter
- D. recovering the pellets of said particulate solid from said chamber.

2. A process according to claim 1 wherein said particulate solid is carbon black.

3. A process according to claim 2 wherein said pelleting liquid is an aqueous molasses solution.

4. A process according to claim 2 wherein said gaseous fluid is pulsatingly introduced through said wall.

5. A process according to claim 2 wherein said gaseous fluid is air.

\* \* \* \* \*

| Example I                      |             |    |
|--------------------------------|-------------|----|
| Feed to Pelleter:              |             |    |
| Carbon Black, No./hr.          | 3000        | 25 |
| Carbon Black Temp., °F         | 250         |    |
| Pelleting Solution, No./hr.    | 3000        |    |
| Pelleting Solution Temp., °F   | 185         |    |
| Pelleter Pressure              | Atmospheric |    |
| Air to Top Jacket:             |             |    |
| Rate, No./hr.                  | 1000        | 30 |
| Inlet Temperature, °F          | 205         |    |
| Outlet Temperature, °F         | 209         |    |
| Inlet Pressure, psig           | 15          |    |
| Steam to Lower Jacket:         |             |    |
| Rate, No./hr.                  | 500*        |    |
| Inlet Temperature, °F          | 230         |    |
| Outlet Temperature, °F         | 220         |    |
| Pulsations/minute              | 30          | 35 |
| Each Pulse                     |             |    |
| On 1.5 seconds                 |             |    |
| Off 0.5 seconds                |             |    |
| Pelleter Shaft Speed, RPM      | 300         |    |
| Wet Pellet Production, No./hr. | 6000        |    |
| Pellet Temperature, °F         | 197         |    |
| Cake Removed, No./hr., est.    | 50          | 40 |

\*About 50 No./hr. pass through apertures.

#### Example II

| Example II                   |             |    |
|------------------------------|-------------|----|
| Feed to Pelleter:            |             |    |
| Carbon Black, No./hr.        | 3000        | 45 |
| Carbon Black Temp., °F       | 250         |    |
| Pelleting Solution, No./hr.  | 3000        |    |
| Pelleting Solution Temp., °F | 185         |    |
| Pelleter Pressure            | Atmospheric |    |
| Air to Top Jacket:           |             |    |
| Rate, No./hr.                | 1000        |    |
| Inlet Temperature, °F        | 200         |    |
| Outlet Temperature, °F       | 204         | 50 |
| Inlet Pressure, psig         | 15          |    |
| Air to Bottom Jacket:        |             |    |
| Rate, No./hr.                | 1000        |    |
| Inlet Temperature, °F        | 230         |    |
| Outlet Temperature, °F       | 220         |    |
| Inlet Pressure, psig         | 15          | 55 |